

# United States Patent [19]

Zoleski et al.

[11] Patent Number: 4,720,350

[45] Date of Patent: Jan. 19, 1988

[54] OXIDATION AND CORROSION  
INHIBITING ADDITIVES FOR RAILWAY  
DIESEL CRANKCASE LUBRICANTS

[75] Inventors: Benjamin H. Zoleski, Beacon;  
Rodney L. Sung, Fishkill; Ronald L.  
O'Rourke, Hyde Park, all of N.Y.

[73] Assignee: Texaco Inc., White Plains, N.Y.

[21] Appl. No.: 851,617

[22] Filed: Apr. 14, 1986

[51] Int. Cl.<sup>4</sup> ..... C10M 129/00

[52] U.S. Cl. ..... 252/51.5 A; 252/51.5 R

[58] Field of Search ..... 252/51.5 A, 51.5 R

[56] References Cited

U.S. PATENT DOCUMENTS

3,184,474 5/1965 Cattu et al. ..... 252/51.5 A  
3,281,356 10/1966 Colemer et al. ..... 252/32.7  
3,331,776 7/1967 Krukziener et al. ..... 252/56

4,219,431 8/1980 Chibnik ..... 252/51.5 A  
4,329,249 5/1982 Fursherg ..... 252/51.5 A  
4,522,736 6/1985 Andress et al. ..... 252/51.5 A  
4,579,674 4/1986 Schlicht ..... 252/51.5 A

Primary Examiner—William R. Dixon, Jr.

Assistant Examiner—Cynthia A. Prezlock

Attorney, Agent, or Firm—Robert A. Kulason; James J. O'Loughlin; Vincent A. Mallare

[57]

## ABSTRACT

A railway diesel crankcase lubricating oil composition for railway diesel engines, containing a mineral lubricating oil, an overbased calcium alkylphenolate and an alkyaryl sulfonate oxidation and corrosion inhibiting amount of a reaction product of alpha-hydroxy omega hydroxy-poly (oxyethylene) poly (oxypropylene) poly (oxyethylene) block copolymer, dibasic acid anhydride and N-alkyl alkylene diamine.

11 Claims, No Drawings



wherein a+c has a value of about 2 to about 80, preferably about 20 to about 40 and more preferably about 70, and b has a value of about 5 to about 70, preferably about 20 to about 30. The molecular weight of the polyol may range from about 800 to about 2000. Examples of the polyols, which may be employed herein, include those listed below in Table I.

TABLE I

- A. The Wyandotte Pluronic L-43 brand of poly (oxyethylene) poly (oxypropylene) poly (oxyethylene) polyol having a molecular weight ( $\bar{M}_n$ ) of 1200 and containing 30 wt.% derived from poly (oxyethylene) and 70 wt.% derived from poly (oxypropylene). In this product, b is 16.6 and a+c is 5.5.
- B. The Wyandotte Pluronic L-63 brand of poly (oxyethylene) poly (oxypropylene) poly (oxyethylene) polyol having a molecular weight ( $\bar{M}_n$ ) of 1750 and containing 30 wt.% derived from poly (oxyethylene) and 70 wt.% derived from poly (oxypropylene). In this product, b is 21.1 and a+c is 11.9.
- C. The Wyandotte Pluronic L-62 brand of poly (oxyethylene) poly (oxypropylene) poly (oxyethylene) polyol having a molecular weight ( $\bar{M}_n$ ) of 1750 and containing 20 wt.% derived from poly (oxyethylene) and 80 wt.% derived from poly (oxypropylene). In this product, b is 24.1 and a+c is 8.
- D. The wyandotte Pluronic L-31 brand of poly (oxyethylene) poly (oxypropylene) poly (oxyethylene) polyol having a molecular weight ( $\bar{M}_n$ ) of 950 and containing 10 wt.% derived from poly (oxyethylene) and 90 wt.% derived from poly (oxypropylene). In this product, b is 14.7 and a+c is 2.2.
- E. The wyandotte Pluronic L-64 brand of poly (oxyethylene) poly (oxypropylene) poly (oxyethylene) polyol having a molecular weight ( $\bar{M}_n$ ) of 1750 and containing 40 wt.% derived from poly (oxyethylene) and 60 wt.% derived from poly (oxypropylene). In this product b is 18.1 and a+c is 15.9.

The amines which may be employed in the present process include polyamines, preferably diamines, which bear at least one primary amine-NH<sub>2</sub> group and at least one substituted primary amine group. The latter may be di-substituted but, more preferably, it is mono-substituted. The hydrocarbon nucleous of the amine may be aliphatic or aromatic, including alkyl, alkaryl, aralkyl, aryl, or cycloalkyl in nature. The preferred amine has the formula



wherein R' is a (C<sub>8</sub>-C<sub>18</sub>) hydrocarbon group and R'' is a (C<sub>1</sub>-C<sub>8</sub>) hydrocarbon group, preferably a (C<sub>2</sub>-C<sub>4</sub>) hydrocarbon group. In the preferred amines, i.e., mono-substituted primary amines, R' may be an alkyl, alkaryl, aralkyl, aryl, or cycloalkyl hydrocarbon group and R'' may be an alkylene, aralkylene, alkarylene, arylene, or cycloalkylene hydrocarbon group.

Illustrative of the preferred N-primary alkylalkylene diamines may include those listed below in Table II.

TABLE II

- A. The Duomeen O brand of N-oleyl-1,3-propane diamine.

- B. The Duomeen S brand of N-stearyl-1,3-propane diamine.
- C. The Duomeen T brand of N-tallow-1,3-propane diamine.
- D. The Duomeen C brand of N-coco-1,3-propane diamine.

The most preferred diamine, R'-NH-R''-NH<sub>2</sub>, is that where the R'' group is propylene, —CH<sub>2</sub>CH<sub>2</sub>CH<sub>2</sub>—, and the R' group is a (C<sub>12</sub>-C<sub>18</sub>) n-alkyl group.

In accordance with the present invention, the process comprises the addition to the hydrocarbon fuel, of a minor deposit-inhibiting amount of, as a deposit-inhibiting additive, a reaction product of (a) a polyol, (b) maleic anhydride, and (c) an N-alkyl-alkylene diamine.

The following example is provided to illustrate the preferred method of preparing the present reaction product and the effectiveness of the product in railway diesel crankcase lubricants. It will be understood that the following example is merely illustrative and not meant to limit the invention in any way.

## EXAMPLE

The reaction, i.e., condensate product is prepared by first reacting maleic anhydride with the prescribed polyol. The reaction of about 1 to about 2 mole, preferably about 1 mole maleic anhydride with about 1 to about 2 moles, preferably about 1.0 mole polyol is preferably carried out in the presence of a solvent. Suitable solvents include hydrocarbons boiling in the gasoline boiling range of about 30° C. to about 200° C. Generally, this will include saturated and unsaturated hydrocarbons having from about 5 to about 10 carbon atoms. Specific suitable hydrocarbon solvents include hexane, cyclohexane, benzene, toluene, and mixtures thereof. Xylene is the preferred solvent. The solvent can be present in an amount of up to about 90 percent by weight of the total reaction mixture. The mixture is heated for 2 hours, then cooled to 60° C. and then add 1 mole of N-alkyl alkylene diamine. The mixture is heated at 100° C. for 2 more hours, whereupon it is filtered and stripped under vacuum.

In a preferred method for preparing the reaction product, the 1 mole maleic anhydride and 1 mole of Pluronic L-43 are combined with the solvent xylene and reacted at a temperature of about 100° C. The reaction mixture is maintained at this temperature for approximately 2 hours. The mixture is then cooled to about 60° C., whereupon the 1 mole of Duomeen-T is added. The new mixture is then reacted at about 100° C. for approximately 2 hours. The reaction product can then be separated from the solvent, using convention means or left in admixture with some or all of the solvent, to facilitate addition of the reaction product to diesel or other diesel lubricants, e.g., marine diesel lubricant. The final reaction product (E) structure (as evidenced by elemental analysis, IR analysis, and NMR analysis) is shown in the illustration below.

In the process illustrated below, initially, maleic anhydride (A) is reacted with a polyol (B) to form an ester of maleic acid (C) then, the ester of maleic acid (C) is reacted with an N-alkyl alkylene diamine (D) to form the condensate product (E) of a polyol, maleic anhydride and an N-alkyl alkylene diamine. Accordingly, the condensate product (E) is recovered.



Wherein  $a+c$  has a value of about 2 to about 80, preferably about 20 to about 40 and more preferably about 70, and  $b$  has a value of from about 5 to about 70, preferably about 20 to about 30;  $\text{R}'$  is a ( $\text{C}_8$ - $\text{C}_{18}$ ) alkyl, alkaryl, aralkyl, aryl or cycloalkyl hydrocarbon group, and  $\text{R}''$  is a ( $\text{C}_1$ - $\text{C}_8$ ) alkylene, aralkylene, alkarylene, or cycloalkylene hydrocarbon group.

The preferred components of the railway diesel crankcase lubricating oil composition of the present invention are those which are effective in a range of from about 0.1 to about 5.0 wt.% based on the total lubricating oil composition. However, it is preferred to employ from about 0.5 to about 2.0 wt.% of the derivative based on the weight of the lubricating oil with the most preferred concentration ranging from about 0.75 to about 1.5 wt.%.

The railway diesel crankcase lubricating oil composition, in other words, comprises

(a) a major portion of a liquid paraffinic mineral oil having a viscosity at 100° C. of about 52.5 SUS minimum, a paraffinic mineral oil having a viscosity at 100° C. of about 75.0 to about 79.0 SUS and a liquid naphthenic mineral oil having a viscosity at 100° C. of about 75.0 to about 80.0 SUS, and

(b) a minor amount of, as an oxidation and corrosion inhibiting agent, a condensate product prepared (as described above) from the reaction of a polyol, maleic anhydride and an N-alkyl alkylene diamine.

The second essential component of the railway diesel crankcase lubricating oil composition of the instant invention is an overbased calcium alkylphenolate, a phenate or a sulfurized overbased calcium alkylphenolate in a sufficient amount to provide a Total Base Number (TBN) ranging from about 3 to about 13 in the finished railway diesel crankcase lubricating oil composition. The increase in viscosity is a measure of the oxidation increase and the metal weight loss is a measure of the corrosion deterioration.

30

#### OIL OXIDATION TEST

The test method involves bubbling 5 liters of oxygen per hour through 300 mls. of test oil composition at 285° F. in which there is immersed a  $1 \times 3 \times 0.06$  inch steel backed copper-lead test specimen, cut from bearing stock. The viscosity of the test oil is measured before and after the 144 hour test period and greater the difference in viscosity, the greater the oxidative deterioration of the instant invention. In addition, the test specimen is weighed before and after the test period and the greater the weight loss of test specimen the greater the corrosion deterioration of the test formulation. Further, the larger the amount of copper, iron and lead moieties found in the oil after test, the greater the oxidative/corrosion deterioration thereof.

The representative Formulations A, B and comparative Formulation C and their oxidation test results are reported below in Table III.

TABLE III

| Oil Code                                                            | Identification | Composition, wt. % | A      | B      | C      |
|---------------------------------------------------------------------|----------------|--------------------|--------|--------|--------|
| Overbased Ca alkaryl sulfonate/phenate <sup>(1)</sup>               |                | 4.10               | 4.10   | 4.10   |        |
| Ca Salt of poly-isobutylene phenol-aldehyde-amine reaction product  |                | 1.46               | 1.46   | 1.46   |        |
| Polyisobutylene                                                     |                | 0.44               | 0.44   | 0.44   |        |
| Branched alkyl ( $\text{C}_{16}$ ) phenol                           |                | 0.88               | 0.88   | 0.88   |        |
| Chlorowax                                                           |                | 0.15               | 0.15   | 0.15   |        |
| SNO-320 <sup>(2)</sup>                                              |                | 19.64              | 19.64  | 20.14  |        |
| SNO-850 <sup>(3)</sup>                                              |                | 30.02              | 30.02  | 30.52  |        |
| 75/80 Pale Oil <sup>(4)</sup>                                       |                | 37.31              | 37.31  | 37.31  |        |
| Low quality marine diesel fuel <sup>(5)</sup>                       |                | 5.00               | 5.00   | 5.00   |        |
| Experimental anti-oxidation, anti-corrosion additive <sup>(6)</sup> |                |                    | 1      |        |        |
| Experimental anti-oxidation anti-corrosion additive <sup>(7)</sup>  |                |                    |        | 1      |        |
| Test Results                                                        |                |                    |        |        |        |
| wt. loss, gm                                                        |                |                    | 0.0078 | 0.0903 | 0.2574 |

TABLE III-continued

| Oil Code                          | A    | B    | C    |
|-----------------------------------|------|------|------|
| Identification Composition, wt. % | 24.2 | 50.1 | 82.0 |

(1) The ratio of sulfonate to phenate is 1:1.

(2) A paraffinic mineral oil having a 40° C. viscosity in the range of 308-350 SUS and a 100° C. viscosity of 52.5 SUS minimum.

(3) A paraffinic mineral oil having a 40° C. viscosity in the range of 800-890 SUS and a 100° C. viscosity in the range of 75.0-79.0 SUS.

(4) A naphthenic pale oil having a 100° C. viscosity in the range of 75-80 SUS.

(5) Low quality marine diesel fuel. (See Attachment I below for specifications).

(6) Reaction product of Pluronic L-43, maleic anhydride and N-tallow-1,3-propane diamine.

(7) Reaction product of Pluronic L-43, maleic anhydride and N-coco-1,3-propane diamine.

## ATTACHMENT I

|                                    |       |
|------------------------------------|-------|
| Density, g/ml 15° C.               | 0.962 |
| Viscosity, CST at 50° C.           | 173   |
| Water content, O/O V/V             | 0.0   |
| Conradson: Carbon residue, O/O M/M | 12.7  |
| Sulphur: O/O M/M                   | 1.47  |
| Ash, O/O M/M                       | 0.06  |
| Vandium: MG/KG                     | 30    |
| Sodium, MG/KG                      | 120   |
| Allminium, MG/KG                   | 16    |
| Silicon, MG/KG                     | 38    |
| Compatability with MGO             | No. 1 |
| Calc. lower heat value, MJ/KG      | 40.63 |

We claim:

1. A railway diesel crankcase lubricant composition comprising a major portion of a diesel lubricating oil and a minor amount of, as an oxidation and corrosion inhibiting agent, a condensate product prepared by the process comprising:

(i) reacting a dibasic acid anhydride of the formula



where R is H,  $\text{CH}_3-$  or  $\text{C}_2\text{H}_5-$ , with a polyol of the formula



where  $a+c$  has a value of about 2 to about 80 and  $b$  has a value of about 5 to about 70; thereby forming an ester of maleic acid;

(ii) reacting said ester of maleic acid with an N-alkyl alkylene diamine, thereby forming the condensate product; and

(iii) recovering said condensate product.

2. The railway diesel crankcase lubricant composition of claim 1, wherein said polyol has a molecular weight ( $\bar{M}_n$ ) ranging from about 800 to about 2000.

3. The railway diesel crankcase lubricant composition of claim 1, wherein said polyol is reacted with a dibasic acid anhydride.

4. The railway diesel crankcase lubricant composition of claim 1, wherein said N-alkyl alkylene diamine has the formula



where R' is a ( $\text{C}_8-\text{C}_{18}$ ) hydrocarbon group and R'' is a ( $\text{C}_1-\text{C}_8$ ) hydrocarbon group.

5. The railway diesel crankcase lubricant of claim 4, where R'' is a ( $\text{C}_2$  to  $\text{C}_4$ ) hydrocarbon group.

6. The railway diesel crankcase lubricant composition of claim 1, wherein the minor amount of oxidation and corrosion inhibiting agent ranges from about 0.1 to about 5.0 weight percent of said lubricant composition.

7. The railway diesel crankcase lubricant composition of claim 6, wherein the minor amount of inhibiting agent ranges from about 0.5 to about 2.0 wt.% of said lubricant composition.

8. The railway diesel crankcase lubricant composition of claim 7, wherein the minor amount of inhibiting agent ranges from about 0.75 to about 1.5 to wt.% of said lubricant composition.

9. The railway diesel crankcase lubricant composition of claim 1, wherein said lubricant composition includes an overbased calcium alkylphenolate, a phenate or a sulfurized overbased calcium alkylphenolate in a sufficient amount to have a Total Base Number ranging from about 3 to about 13.

10. A railway diesel crankcase lubricant composition comprising:

(a) a major portion of a liquid paraffinic mineral oil having a viscosity at 100° C. of about 52.5 SUS minimum, a paraffinic mineral oil having a viscosity at 100° C. of about 75.0 to about 79.0 SUS and a liquid naphthenic mineral oil having a viscosity at 100° C. of about 75.0 to about 80.0 SUS,

(b) a minor amount of, as an oxidation and corrosion inhibiting agent, a condensate product of the process comprising:

(i) reacting a polyol



where  $a+c$  has a value of about 2 to about 80 and  $b$  has a value of about 5 to about 70, with a dibasic acid anhydride of the formula



where R is H,  $\text{CH}_3-$  or  $\text{C}_2\text{H}_5-$ , thereby forming an ester of maleic acid;

(ii) reacting said ester of maleic acid with an N-alkyl alkylene diamine



where R' is a ( $\text{C}_8-\text{C}_{18}$ ) hydrocarbon group and R'' is a ( $\text{C}_1-\text{C}_8$ ) hydrocarbon group, thereby forming a condensate product.



(iii) recovering said condensate product.

11. A diesel crankcase lubricant composition comprising: 10

(a) a major portion of a liquid paraffinic mineral oil having a viscosity at 100° C. of about 52.5 SUS minimum, a paraffinic mineral oil having a viscosity at 100° C. of about 75.0 to about 79.0 SUS and a liquid maphthenic mineral oil having a viscosity at 100° C. of about 75.0 to about 80.0 SUS, 15

(b) about 1 wt.% of an oxidation and corrosion inhibiting condensate product of the process comprising:

(i) reacting a dibasic acid anhydride of the formula <sup>20</sup>



where R is H,  $\text{CH}_3-$  or  $\text{C}_2\text{H}_5-$ , with a polyol of the formula

$$\text{HO}(\text{CH}_2\text{CH}_2\text{O})_a(\text{CHCH}_2\text{O})_b(\text{CH}_2\text{CH}_2\text{O})_c\text{H};$$

$\text{CH}_3$

where  $a+c$  has a value of about 2 to about 80 and  $b$  has a value of about 5 to about 70, thereby forming an ester of maleic acid



(ii) reacting said ester of maleic acid with N-tallow-1,3-propane diamine, thereby forming a said condensate product



(iii) recovering said condensate product.

50

55

60

65